

## UNITED STATES PATENT OFFICE

2,613,183

## SULFURIZED ADDITIVES FOR LUBRICATING COMPOSITIONS

Abraham D. Kirshenbaum, Union, and James M. Boyle, Bayonne, N. J., assignors to Standard Oil Development Company, a corporation of Delaware

No Drawing. Application August 19, 1949,  
Serial No. 111,343

19 Claims. (Cl. 252—46.7)

1.

The present invention relates to improvements in sulfurized additives for lubricating compositions, to a method of preparing such additives, and to compositions containing them. In particular, the invention relates to additive compositions prepared by treating monocyclic terpenic hydrocarbons and related materials having a similar unsaturated non-aromatic ring structure, to incorporate sulfur, phosphorus and chlorine or other halogen therein, thereby to convert such compositions into extreme pressure agents or oxidation or corrosion inhibitors for lubricating oils and greases.

As is well known in the art, ordinary hydrocarbon oils, e. g., lubricating oils derived from petroleum, are good lubricants for many purposes but are deficient in strength of lubricating film when subjected to high unit pressures. The same is true of the synthetic oils, i.e., esters of dibasic acids and the like. Thus, in the lubrication of antifriction bearings, gearing, and other mechanical parts subjected to high unit pressures, the untreated lubricating oils and greases prepared therefrom are frequently inadequate to prevent metal-to-metal contact and consequently injury to metal surfaces. In the lubrication of parts which are subjected both to extremely high pressures and to sliding friction, the need for a film-strengthening or oil-replacing lubricating additive becomes particularly imperative. A well known example is the lubrication of hypoid gears in automotive vehicles. Unit pressures on contacting elements of such gears sometimes attain the magnitude momentarily of a hundred thousand pounds per square inch or more. Such gears, moreover, are subject to sliding contact as well as, or as distinguished from, true rolling contact, and, hence, they are particularly subject to severe and intolerable wear unless protected by an adequate lubricant.

Numerous suggestions have been made in the prior art for using chlorinated, sulfurized, and/or phosphorized products as such extreme pressure additives to mineral base and other oily lubricants. It is well known that certain chlorinated products, e. g., chlorinated hydrocarbons, are capable of providing a protective film of metal chloride, apparently a mono-molecular film, by reacting momentarily with metal elements such as gears which come into contact under heavy unit loads and under conditions giving rise to instantaneous high temperatures over limited areas. Likewise, certain prior art compositions containing sulfur or phosphorus, or both, or containing chlorine or other halogen with either sul-

fur or phosphorus, or both, have been suggested as having good load-bearing properties under severe operating conditions. In general, these prior art compounds have been prepared on the theory that the halogen, and/or sulfur, and/or phosphorus, reacts with the metal itself and forms an extremely thin (supposedly mono-molecular) but adequately protective film thereon to prevent seizure and damage to the contacting metal elements being lubricated until the normal oil film, disrupted by the heavy impact, can be reestablished. Some of such materials have been accepted commercially by the industry. Some others have not been commercially successful because of their cost or because of operating deficiencies under extremely severe conditions.

The present invention is based upon the discovery that a relatively inexpensive and yet highly effective extreme pressure additive may be prepared by first treating a monocyclic terpene, such as limonene, dipentene, terpinoline, alpha terpinene, and the like, with a sulfur chloride and then with a phosphorus sulfide to incorporate all three elements, sulfur, chlorine, and phosphorus into the reaction product. These terpenes have the typical formulas



and



and appear to be structurally, if not actually, polymers of isoprene. They are characterized by the unsaturated non-aromatic ring and the branched aliphatic group attached. Other materials having the same general characteristics also may be used.

While any of the sulfur chlorides may be used to treat the terpenes, the monochloride  $S_2Cl_2$  is preferred. For the phosphorus sulfide, the sesquisulfide  $P_4S_3$  is preferred because it tends to add more phosphorus and less sulfur and thereby to reduce the corrosivity of the reaction product towards metals. Where this consideration is not of too great importance, the other phosphorus sulfides  $P_2S_5$ , etc., may be used in lieu of  $P_4S_3$ .

According to the present invention, an inexpensive lubricating oil additive is prepared preferably by first partially reacting the monocyclic

terpene (diolefin), e. g., dipentene, with sulfur chloride and thereafter reacting the resulting product with the phosphorus sulfide. The sulfur chloride is preferably added in such quantities and reacted under such conditions that approximately one of the double bonds of the terpene, on the average, is saturated thereby. The phosphorus sulfide is then introduced and it reacts largely with the second double bond giving a single compound containing all three of the elements, phosphorus, sulfur and chlorine. The quantity of phosphorus sulfide used, however, is considerably less than that required to saturate the second double bond of all the terpene molecules. Apparently, some polymerization takes place. In general, only a small amount of phosphorus sulfide is used where the product is intended as an extreme pressure additive. Larger proportions may be used where the product is to be used in very small quantities as an oxidation or corrosion inhibitor.

The invention will be more fully understood by reference to the following specific examples.

*Example I*

797 g. (475 c. c.) of sulfur monochloride was added to 1 liter (841 g.) of special commercial "dipentene" (from Hercules Powder Co.). This special dipentene had the following composition: 6%  $\alpha$ -pinene, 7%  $\alpha$ -terpineol, 10% para cymene, 31% dipentene, 39% terpinolene, 5%  $\Delta 2,4(8)$  para menthadiene, 2% residue. The para cymene appears to be the only non-reactive component. Therefore, only about 90% of the special dipentene takes part in the reaction. The sulfur monochloride was introduced into the terpene at a rate of 15-20 c. c. per minute at 75-100° C. with constant stirring. After all the  $S_2Cl_2$  was added, the product was heated at 75-100° C. for  $\frac{3}{4}$  to 1 hour. The  $S_2Cl_2$ -treated "dipentene" (mixture) gave an analysis of 17.4% chlorine and 23.7% sulfur.

150 g. of the  $S_2Cl_2$ -treated "dipentene" was diluted with 150 g. of a naphthenic lube distillate of grade SAE 30. 10 g. of  $P_4S_3$  was added and heated with stirring for one hour at 125-150° C.  $HCl$  was liberated. After one hour of heating, there were added 25 g. "Lorol B" alcohol, which is a well known commercial mixture of  $C_{10}$  to  $C_{18}$  primary alcohols, predominantly about  $C_{12}$ , prepared from coconut oil, and heating was continued for 15 minutes more. The product was blown with nitrogen gas and filtered through a commercial filter aid known as "Hyflo." The final product contained

3.74% chlorine  
13.65% sulfur  
1.68% phosphorus

The following blend of the above product was made:

2.5 weight per cent product  
7.5 weight per cent chlorinated wax (40 weight per cent chlorine)  
90.0 weight per cent of a mixture of about equal parts of a steam refined Pennsylvania cylinder oil having a viscosity of 220 S. S. U. at 210° F. and a Mid-Continent acid refined oil having a viscosity of 50 S. S. U. at 210° F.

This blend gave the following results:

Timken machine test: Pass 33 lbs.  
SAE machine test: Pass 300+  
Copper strip test: Pass

*Example II*

150 g. (1.45 mols) of  $SCl_2$  was added dropwise (2.5 g./min.) to 210 g. (1.55 mols) of special dipentene (Hercules) with constant agitation. The temperature was kept between 40° and 60° C. by means of a water and ice bath. After all the  $SCl_2$  was added, the product was first kept for  $\frac{1}{2}$  hour at about 20° C. and then for one hour at 75° to 100° C. 300 g. of mineral base oil of 55 S. S. U. viscosity at 210° F. and 20 g. of  $P_4S_3$  were then added and the mixture was heated for one hour at 125-150° C. Then 50 g. of "Lorol B" alcohol were added and heated at 125-150° C. for  $\frac{1}{4}$  hour more. The product was blown with nitrogen gas to remove  $HCl$  and  $H_2S$  and light ends, and filtered through "Hyflo."

The product had the following analysis:

4.08% chlorine  
9.08% sulfur  
1.82% phosphorus

The following blend was made and tested for extreme pressure properties:

25 2.5 weight per cent of product  
7.5 weight per cent chlorinated wax (40 weight per cent chlorine)  
90.0 weight per cent of a mixture of a steam refined Pennsylvania cylinder oil having a viscosity of 220 S. S. U. at 210° F. and a Mid-Continent acid refined oil having a viscosity of 50 S. S. U. at 210° F.

The blend gave the following results:

35 Timken machine test: Pass 33 lbs.  
SAE machine test: Pass 280 lbs.  
Copper strip test: Pass

It will be understood that the general procedure described above is applicable to various combinations of materials, e. g., the dichloride  $SCl_2$  may be used in lieu of  $S_2Cl_2$ , as shown in Example II. The quantity of the sulfur chloride should be such that approximately one of the double bonds in the terpene is saturated. When the monochloride  $S_2Cl_2$  is employed, about one mol of  $S_2Cl_2$  per mol of terpene gives good results. If the proportion is much greater, very viscous products are obtained. However, in the case of the dichloride  $SCl_2$ , the mol ratio of  $SCl_2$  to terpene may be 1/1 or as high as 2/1. The reaction temperature when employing  $S_2Cl_2$  can be between 60° and 125° C., preferably from 75° to 100° C. When the dichloride is employed, it should be added at a lower temperature, such as 30° to 60° C. to avoid a violent reaction, and thereafter the reaction can be completed at a higher temperature such as 75° to 100° or 125° C. The addition reaction is substantially complete in from  $\frac{1}{2}$  to 1 $\frac{1}{2}$  or 2 hours. The phosphorus sulfide is then added, preferably in an amount which will give a product containing from about 0.04 to about 4.0 weight per cent of phosphorus on the 100% undiluted basis. This range corresponds to reacting from about 0.000875 to about 0.0875 mols  $P_4S_3$  (containing 0.0035 to 0.35 atoms of phosphorus) per mol of  $S_2Cl_2$ -treated terpene. The reaction is conducted at a temperature of 100° to 175° C., preferably from 125° to 150° C., until the reaction is substantially completed, requiring a time of from about  $\frac{1}{4}$  to 2 hours. In general, the molar proportions of phosphorus sulfide will run between about 0.001 and 0.1.

The finished lubricant preferably contains a quantity of a conventional chlorinated hydro-

carbon, such as chlorinated wax, chlorinated kerosene or other halogenated hydrocarbon of long chain aliphatic structure. The halogenated hydrocarbon is combined with a smaller quantity of the dipentene or other treated terpene. A preferred composition range is from about 80-95% of the oil or other lubricant, 4 to 15% of the halogenated hydrocarbon and 1 to 5% of the treated terpene. Specifically, the preferred proportions are about 90% of the lubricant, preferably mineral lubricating oil, with about 7.5% of the halogenated hydrocarbon and about 2.5% of the treated terpene.

In many cases, it is not necessary to use an auxiliary additive, such as the chlorinated hydrocarbon referred to above. Where extreme pressure requirements are not excessive, the terpene treated first with a sulfur chloride and subsequently with a phosphorus sulfide is quite adequate by itself. When the single additive is used, it preferably comprises from 2 to 20% of the weight of the total composition. More specifically, proportions of about 5 to 12% will ordinarily be used.

The present invention comprehends both the treated dipentene as a new product per se together with process for its treatment, and also the lubricating composition containing the treated dipentene or other terpene as an additive. Lubricating compositions containing such additive may be of mineral or synthetic oil base, or both. They may also contain other conventional materials such as antioxidants, viscosity index improvers, thickeners, tackiness agents, pour point depressors, and the like. The additive itself may be used in straight mineral oils or in blends with synthetic oils and also in lubricating greases and lubricating compositions of widely varying consistencies.

While the treatment with sulfur chlorides and phosphorus sulfides has been described with particular reference to terpenes such as dipentene, it is applicable in general to hydrocarbons, and esters, acids, alcohol and ketonic derivatives thereof having the general unsaturated non-aromatic structure pointed out above. Thus it may be applied to abietic acid and lower alkyl esters thereof, such as "Abalyn" (methyl abietate), "Hercolyn" (hydrogenated abietic esters), and the like.

What is claimed is:

1. An extreme pressure additive composition for lubricants consisting essentially of the reaction product of about 1 molar proportion of a monocyclic terpene with about 1 to 2 molar proportions of a sulfur chloride, the quantity of said sulfur chloride being substantially sufficient to saturate one double bond in said terpene, said reaction product being further reacted with about 0.001 to 0.1 molar proportion of phosphorus sulfide at a temperature of 100° to 175° C.

2. Composition according to claim 1 wherein the sulfur chloride is  $S_2Cl_2$ .

3. Composition according to claim 1 wherein the sulfur chloride is  $SCl_2$ .

4. A lubricating composition consisting essentially of 80 to 95% by weight of mineral base lubricating oil, 1 to 5% of the reaction product of one molar proportion of a monocyclic terpene treated first with about 1 to 2 molar proportions of a sulfur chloride and reacted thereafter with about 0.001 to about 0.1 molar proportions of a phosphorus sulfide at a temperature of 100° to 175° C., and 4 to 15% of a halogenated long

chain aliphatic hydrocarbon, said sulfur chloride being effective to substantially saturate an average of about one double bond per terpene molecule and said phosphorus sulfide being effective to partially saturate, on the average, the second double bond of the terpene molecule.

5. A lubricating composition according to claim 4 wherein the sulfur chloride is  $S_2Cl_2$ .

6. A lubricating composition according to claim 10 4 wherein the sulfur chloride is  $SCl_2$ .

7. A lubricating composition consisting essentially of about 90% by weight of mineral base lubricating oil, 7.5% of chlorinated wax, and 2.5% of a reaction product of a monocyclic terpene, treated first with about 1 to 2 mols per mol of said terpene of a sulfur chloride and treated thereafter with about 0.001 to 0.1 mols of a phosphorus sulfide at a temperature of 100° to 175° C.

8. Composition according to claim 1 wherein the terpene is dipentene.

9. Composition according to claim 4 wherein the terpene is dipentene.

10. Composition according to claim 7 wherein the terpene is dipentene.

11. A method of preparing an extreme pressure additive for lubricants and the like, which consists in first reacting 1 molar proportion of a monocyclic terpene with about 1 to 2 molar proportions of sulfur chloride at a temperature between about 60° and 125° C., the quantity of sulfur chloride being approximately that required to saturate one double bond of the terpene, and thereafter reacting the treated dipentene with about 0.001 to about 0.1 molar proportions of phosphorus sulfide at a temperature between about 125° and 150° C. for a period of  $\frac{1}{4}$  to 2 hours to partially saturate a second double bond of said terpene.

12. A method of preparing a sulfur and phosphorus-containing organic compound which comprises treating a non-aromatic mono-cyclic terpenic  $C_{10}$  material having a six-membered unsaturated ring with approximately one to two molar equivalents of a sulfur chloride at a temperature of 60° to 125° C. for about  $\frac{1}{2}$  to 2 hours, and subsequently treating the sulfur chloride-treated product with about 0.001 to 0.1 molar proportions of phosphorus sulfide at a temperature of 100° to 175° C. for about  $\frac{1}{4}$  to 2 hours.

13. Method according to claim 12 wherein the organic material is a terpene comprising a substantial proportion of dipentene.

14. Method according to claim 12 wherein the sulfur chloride is  $SCl_2$ .

15. Method according to claim 12 wherein the sulfur chloride is  $S_2Cl_2$ .

16. Method according to claim 12 wherein the phosphorus sulfide is  $PS_3$ .

17. The process which comprises treating a substantially mono-cyclic terpene composition comprising dipentene with 1 to 2 molar proportions, based on said terpene composition, of a sulfur chloride of one to two chlorine atoms per sulfur atom at a temperature between 60° and 125° C. for  $\frac{1}{2}$  to 2 hours and thereafter treating the reaction product with about 0.001 to 0.1 molar proportion of  $PS_3$  at 125° to 150° C. for  $\frac{1}{4}$  to 2 hours.

18. As a new composition of matter, the reaction product of a molar proportion of substantially mono-cyclic terpene composition containing a substantial proportion of dipentene treated first with about one to two mols of sulfur chloride having one to two chlorine atoms per sulfur atom

at a temperature of between 60° and 125° C., for a period of  $\frac{1}{2}$  to 2 hours, and subsequently treated with 0.001 to 0.1 mols of phosphorus sulfide at a temperature of 125° to 150° C. for  $\frac{1}{4}$  to 2 hours.

19. Composition according to claim 18 to which is added 80 to 98%, based on the weight of the total composition, of a mineral base lubricating oil.

ABRAHAM D. KIRSHENBAUM.  
JAMES M. BOYLE.

## REFERENCES CITED

The following references are of record in the file of this patent:

## UNITED STATES PATENTS

| Number    | Name     | Date          |
|-----------|----------|---------------|
| 2,268,232 | Whittier | Dec. 30, 1941 |
| 2,307,183 | Zimmer   | Jan. 5, 1943  |
| 2,413,648 | Ott      | Dec. 31, 1946 |
| 2,468,520 | Sproule  | Apr. 26, 1949 |